

Dec. 21, 1948.

E. B. KNOTT ET AL  
PHOTOGRAPHIC PROCESSES AND LIGHT-SENSITIVE  
ELEMENTS THEREFOR  
Filed Aug. 1, 1947

2,456,955



EDWARD BOWES KNOTT  
GUY WILLIAM WILLIS STEVENS  
INVENTORS

BY *N. M. Perrins*  
*Daniel J. Drayne*  
ATTORNEYS

## UNITED STATES PATENT OFFICE

2,456,955

## PHOTOGRAPHIC PROCESSES AND LIGHT-SENSITIVE ELEMENTS THEREFOR

Edward Bowes Knott and Guy William Willis Stevens, Harrow, Wealdstone, England, assignors to Eastman Kodak Company, Rochester, N. Y., a corporation of New Jersey

Application August 1, 1947, Serial No. 765,634  
In Great Britain June 2, 1944

12. Claims. (Cl. 95—5)

1

This invention relates to photographic processes and materials therefor. This invention is a modification of that described and claimed in our copending application Serial No. 765,636, filed August 1, 1947. In said application Serial No. 765,636, we have described certain methods and materials using two different kinds of silver salt emulsions, designated therein as emulsions of type I and emulsions of type II, so constituted and arranged on a single support that each of them can be selectively exposed, and the modification in which this requirement regarding selective exposure can be dispensed with in which case the emulsions have differing gammas.

We have now found that said requirement can be dispensed with even when the emulsions give the same gamma.

The present invention provides the method of producing a photographic image of an object or image wherein a light-sensitive material comprising a silver salt emulsion of type I and a silver salt emulsion of type II, both of the same gamma and coated either as superimposed layers or mixed, i. e., inseparably combined and extending over the same area on a single support, is exposed to said lighted object or image, thereby exposing both emulsions simultaneously, and the exposed material is developed first in a "surface" developer and then in an "internal" developer.

Type I emulsions are those which upon exposure to light form the latent image mostly inside the silver salt grains. These emulsions after exposure to light can be developed in "internal" developers. Type II emulsions are those which upon exposure to light form surface latent images. These emulsions after exposure to light can be developed in either "internal" or "surface" developers.

Developers for developing such latent images are as follows:

## FORMULA I

## "SURFACE" DEVELOPER

|                           |       |      |
|---------------------------|-------|------|
| p-Hydroxyphenylglycine    | grams | 10   |
| Sodium carbonate (cryst.) | do    | 100  |
| Water to                  | ccs   | 1000 |

Development time 4 minutes at 20° C.

2

## FORMULA II (a)

## "INTERNAL" DEVELOPER

|                                 |       |      |
|---------------------------------|-------|------|
| Hydroquinone                    | grams | 15   |
| N-methyl-p-aminophenol sulphate | do    | 15   |
| Sodium sulphite, anhy.          | do    | 50   |
| Potassium bromide               | do    | 10   |
| Sodium hydroxide                | do    | 25   |
| Sodium thiosulphate (cryst.)    | do    | 20   |
| Water to                        | ccs   | 1000 |

Development time 3 minutes at 20° C.

## FORMULA II (b)

## "INTERNAL" DEVELOPER

|                                 |       |      |
|---------------------------------|-------|------|
| Hydroquinone                    | grams | 12   |
| N-methyl-p-aminophenol sulphate | do    | 3    |
| Sodium sulphite (cryst.)        | do    | 90   |
| Potassium bromide               | do    | 4    |
| Sodium carbonate (cryst.)       | do    | 150  |
| Sodium thiosulphate (cryst.)    | do    | 20   |
| Water to                        | ccs   | 1000 |

Development time 4 minutes at 20° C.

## FORMULA III

## COMMERCIAL DEVELOPER

This is the same as Formula II (b), but omitting the sodium thiosulphate.

Formula II (a) is a more energetic developer than Formula II (b) so that it usually gives a higher effective speed and a higher contrast than Formula II (b) but is often not so convenient, since it has a higher tendency to aerial oxidation and to give fog.

While in this specification we have described our invention partly in regard to a theory of internal and surface latent images, the correctness or otherwise of such theory, is not essential to the successful working of the invention; it being only necessary to choose the emulsions according to the tests herein after given.

The present invention employs the following types of emulsions:

## TYPE I

45 These are the emulsions which will develop (after exposure to light) in internal developers of the kind given in at least one of Formulae II (a) and II (b), but will not develop or only slightly develop in Formula III or in Formula I, i. e., the surface developers.

(1) *Normal range of exposures*

As measured according to normal photographic testing technique, when a test layer of the type I emulsion is coated on a transparent support (e. g. glass) and the layer is exposed to a light intensity scale the whole of which is exposed for some fixed time between  $1/100$  and 1 second and is developed in the internal developer II (a) the transmitted density obtained at any point along the  $\log_{10}E$  axis over a density range of 3.0 starting from the threshold of the curve ( $D=0.1$  above fog) should be at least 5 times, and preferably at least 10 times the transmitted density obtained when an identical test layer of the emulsion is developed with the surface developer of Formula I or preferably III, the measurements of density being made at the corresponding (i. e. the same) points on the  $\log_{10}E$  axis; as indicated, the best (i. e. preferred) emulsions are those giving the highest density ratios and the very best (i. e. most preferred) emulsions can be selected with greater certainty by substituting Formula II (b) for II (a).

(2) *Small range of exposures*

For this purpose the emulsion need not conform to such a rigid requirement, for instance for making a tone correcting mask, but it is sufficient if in the above test the upper limit of 3.1 is substituted by an upper limit of 1.0.

## TYPE II

These are the emulsions which when exposed to a light intensity scale, the whole of which is exposed for some fixed time between  $1/100$ th and 1 second, will develop normally in Formulae I and III as well as in Formulae II (a) and II (b). As measured according to normal photographic testing technique, when a test layer of the emulsion is coated on a transparent support (e. g. glass) and the layer is exposed to a light intensity scale the whole of which is exposed for some fixed time between  $1/100$  and 1 second and is developed in the internal developer II (b), the transmitted density obtained at any point along the  $\log_{10}E$  axis of the curve between the density range of 0 to 3.0, preferably 0 to 2.0, does not exceed the transmitted density obtained when an identical test layer of the emulsion is developed in Formula III, the measurements of density being made at the same points on the  $\log_{10}E$  axis of the curve.

Since Formula III contains sodium sulphite and Formula I is free from sulphite, and sulphite is known to have some solvent action on silver chloride and bromide (although very little on silver iodide), it is apparent that when making any of the above measurements on an emulsion to obtain, with a high degree of precision, information on the amount of surface latent image given by such emulsion, it is important to use Formula I.

As will be apparent hereinafter, in performing the invention a small amount of development of the internal latent image is of no real consequence for practical purposes, it may be advisable to employ Formula III, since this developer is not only less liable to aerial oxidation but gives better density in the image produced by the development of the type II emulsion.

It is to be noted that an "internal" developer is necessarily capable of developing not only a latent image inside grains but also of developing a latent image on the surface of grains (whether

such grains contain internal latent image or not) and also of carrying on the development of a surface latent image which has previously been only partly developed.

- 5 It is also to be noted that where a "surface" developer is employed to develop a surface latent image, then all grains which are thereby fully developed cannot be subsequently developed at all in an "internal" developer.
- 10 Gamma can be measured as set forth in British Patent 541,510 and as used herein means the average slope of the characteristic H and D curve between the densities of 0.4 to 1.6. In measuring gamma, development is done at  $68^{\circ}$  F. for  $1\frac{1}{2}$  minutes in the following solution:

|                               |       |                                                                    |
|-------------------------------|-------|--------------------------------------------------------------------|
| N-methyl-p-aminophenol sul-   | grams | 2.2                                                                |
| phate                         | do    | 150.0                                                              |
| Sodium thiosulphate, crystals | do    | 17.0                                                               |
| Hydroquinone                  | do    | 175.0                                                              |
| 20 Sodium carbonate, crystals | do    | 2.8                                                                |
| Potassium bromide             | do    | 1000                                                               |
| Water to                      | ccs   | (This solution is diluted with an equal part of water before use.) |

- 25 The "surface" developer may be for instance a colour-forming developer and the "internal" developer may be a non-colour forming developer, or vice versa, or both developers may be colour developers, for example if one developer gives a yellow coloured image and the other developer gives a cyan (blue-green) coloured image, the finished result will be of green colour and the amount of yellow and the amount of cyan can be conveniently controlled to give any particular shade of green desired, from a very yellowish coloured green to a rather bluish coloured green.

This kind of material is useful in the production of coloured masks for use in colour photographic reproduction where it is desired that the coloured mask should comprise two superimposed images being records of the same colour sensation but of different colours; coloured masks which comprise such images and their use have 40 been described in British Patent No. 568,440. For instance, the material according to the present invention can be made with emulsions both sensitive to red light and after exposure to a multi-coloured original, the one emulsion can be developed with a "surface" developer containing a colour coupler giving a minus blue (yellow) image and then the other emulsion with an "internal" developer containing a colour coupler giving a minus green (magenta) image, the developed silver being subsequently removed in the usual way. When such a combined image is used as a mask in reproducing said original, the minus blue image compensates for the undesired absorption of blue light by the cyan (blue-green) 45 image in the original or in the reproduction or both; similarly the minus green image compensates for the undesired absorption of green light by the cyan image in the original or in the reproduction or both. Similarly both the layers may have a colour sensitivity other than red and developed to other colours just as for the two layers described in British Patent No. 568,440. Although this method of making a mask in two colours involves two development steps it has the advantage over methods involving only one step that the development of each colour can be separately watched and controlled so as to give more easily and exactly the relative depths of 50 colours required. Moreover the two emulsions

can with advantage be coated as a mixture in a single layer.

The accompanying drawing shows a flow-diagram which depicts graphically one embodiment of our invention, viz. the production of a coloured mask as described above. At B is shown a support coated with a red sensitive layer of photographic silver halide emulsion which forms surface latent image and coated on such first emulsion layer, a red sensitive layer of photographic silver halide emulsion which forms latent image mostly inside the silver halide grains, both emulsion layers having the same gamma. Upon exposing this sensitive element to the coloured original shown at A with red light, negative latent image corresponding to the red portion of the coloured original is formed in both emulsion layers as shown to C. Upon developing the whole element in a "surface" colour developer containing a colour coupler giving a minus blue (yellow) image, the upper emulsion layer which contains internal latent image is not developed, while yellow image (from which developed silver is subsequently removed) is formed in the lower emulsion layer as shown at D. Upon developing the element in an "internal" colour developer containing a colour coupler giving a minus green (magenta) image, magenta image (from which developed silver is subsequently removed) is formed in the upper emulsion layer, as shown at E, thus providing a coloured mask which can be used in reproducing said original.

As another illustration the invention is also useful in the production of motion picture sound films, that is to say films having a series of pictures and also a sound track alongside the pictures. In some methods of sound recording and reproduction it is desirable that the gamma of the sound should be lower than that of the pictures. If the material of the present invention is exposed to produce therein latent images of pictures and sound track (side by side) then both can be first developed in a surface developer whereafter the picture areas only can be developed further in an "internal" developer by roller application of such developer to such areas only. Then the film is fixed and washed in the usual way. This will give a greater gamma in the picture areas than in the sound track.

In the present invention the two emulsions may or may not have the same speed according to the results desired or the purpose for which it is to be used. This applies for instance to the two illustrations given above. When the emulsions have different speeds as measured by the exposure which gives a density of 0.2 when developed in the "surface" and "internal" developers referred to above, the material can be used to give a convenient control of the strength of the developed image when the proper exposure is difficult to determine with accuracy. For instance the speed of the type I emulsion can be made greater (say three or five times) than that of the type II emulsion. Such a material can be used for exposure in a camera (or otherwise) and is so exposed for a time which is estimated (by guesswork) to be correct for the type II emulsion. The exposed material is then immersed in a "surface" developer. If the estimate was in fact satisfactory, then the "surface" developer will produce a satisfactory image, but if the estimate was only say one third that of the correct exposure for the type II emulsion then little or no image will develop therein, and in this case the material can then be immersed in an "internal" developer

wherein the Type I emulsion will develop to give an image, which is at least more satisfactory.

Alternatively the type II emulsion can be of greater speed (say five times) than the type I and again first developed in a "surface" developer; in this case if the first developed image in the type II emulsion is unsatisfactory, namely overexposed, it can be bleached out by a silver removing bath (e. g. a bichromate bath) and then the image in the type I emulsion can be developed by means of an "internal" developer. This is useful in the case of camera exposures where the lighting conditions are such that the operator may tend to err on the overexposure side.

10 The preparation of emulsions of type I and type II is described in our copending application Serial No. 765,636, filed August 1, 1947 except it should here be pointed out that there is no great difficulty in making the two emulsions so as to give the same gamma in the sense stated above, for instance an easy way is first to make a type I emulsion of about the desired gamma, then ascertain its gamma accurately, and finally prepare a type II emulsion which during its preparation 15 can be tested and adjusted as is commonly done in the art until it has the same gamma as the type I.

15 The preparation of developers, including colour developers suitable for developing type I and type II emulsions is described in our copending application Serial No. 765,636, filed August 1, 1947.

20 This application is a continuation-in-part of our copending application Serial No. 589,095, filed April 18, 1945.

25 35 What we claim as our invention and desire to be secured by Letters Patent of the United States is:

30 1. The method of selectively producing photographic images in a photographic material containing, inseparably combined and extending over the same area on a single support, two photographic emulsions having the same gamma, one of said emulsions being a light-sensitive silver salt photographic emulsion (I) a test layer of 35 which coated on a transparent glass support upon exposure to a light intensity scale for a fixed time between  $\frac{1}{100}$  and 1 second and development for 3 minutes at 20° C. in the following developer (IIa):

|    |                                 |            |      |
|----|---------------------------------|------------|------|
| 50 | Hydroquinone                    | -----grams | 15   |
|    | N-methyl-p-aminophenol sulphate | do         | 15   |
|    | Sodium sulphite, anhydrous      | do         | 10   |
|    | Potassium bromide               | do         | 10   |
| 55 | Sodium hydroxide                | do         | 25   |
|    | Sodium thiosulphate, crystals   | do         | 20   |
|    | Water to                        | ccs        | 1000 |

55 gives a transmitted density at any point along the  $\log_{10}E$  axis, over a range of 1.0 starting from the threshold of the characteristic curve beginning at a density of 0.1 above fog, at least 5 times the transmitted density obtained when an identical test layer of the emulsion is developed for 4 minutes at 20° C. in the following developer (I):

|    |                            |            |      |
|----|----------------------------|------------|------|
| 60 | p-Hydroxyphenylglycine     | -----grams | 10   |
|    | Sodium carbonate, crystals | do         | 100  |
|    | Water to                   | ccs        | 1000 |

65 70 the measurements of density being made at the same points on the  $\log_{10}E$  axis, and the other of said emulsions being a light-sensitive silver salt photographic emulsion (II) a test layer of which coated on a transparent glass support upon exposure to a light intensity scale for a fixed time between  $\frac{1}{100}$  and 1 second and development

for 4 minutes at 20° C. in the following developer (IIb):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Sodium thiosulphate, crystals   | do    | 20   |
| Water to                        | ccs   | 1000 |

gives a transmitted density at any point along the  $\log_{10}E$  axis of the curve between the range of 0 to 2.0 which does not exceed the transmitted density obtained when an identical test layer of the emulsion (II) is developed for 4 minutes at 20° C. in the following developer (III):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate                | do    | 150  |
| Water to                        | ccs   | 1000 |

the measurements of density being made at the same points on the  $\log_{10}E$  axis of the curve, comprising simultaneously exposing the aforesaid emulsions to a lighted object or image, then treating the whole material with a developer which develops substantially only the latent image which is developable by developer (III) and then developing the whole material in a developer which develops the latent image which is developable by developer (IIa).

2. The method of selectively producing photographic images in a photographic material containing, inseparably combined and extending over the same area on a single support, two photographic emulsions having the same gamma, one of said emulsions being a light-sensitive silver salt photographic emulsion (I) a test layer of which coated on a transparent glass support upon exposure to a light intensity scale for a fixed time between  $\frac{1}{100}$  and 1 second and development for 3 minutes at 20° C. in the following developer (IIa):

|                                 |       |      |
|---------------------------------|-------|------|
| Hydroquinone                    | grams | 15   |
| N-methyl-p-aminophenol sulphate | do    | 15   |
| Sodium sulphite, anhydrous      | do    | 10   |
| Potassium bromide               | do    | 10   |
| Sodium hydroxide                | do    | 25   |
| Sodium thiosulphate, crystals   | do    | 20   |
| Water to                        | ccs   | 1000 |

gives a transmitted density at any point along the  $\log_{10}E$  axis, over a range of 3.0 starting from the threshold of the characteristic curve beginning at a density of 0.1 above fog, at least 5 times the transmitted density obtained when an identical test layer of the emulsion is developed for 4 minutes at 20° C. in the following developer (I):

|                            |       |      |
|----------------------------|-------|------|
| p-Hydroxyphenylglycine     | grams | 10   |
| Sodium carbonate, crystals | do    | 100  |
| Water to                   | ccs   | 1000 |

the measurements of density being made at the same points on the  $\log_{10}E$  axis, and the other of said emulsions being a light-sensitive silver salt photographic emulsion (II) a test layer of which coated on a transparent glass support upon exposure to a light intensity scale for a fixed time between  $\frac{1}{100}$  and 1 second and development for 4 minutes at 20° C. in the following developer (IIb):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Sodium thiosulphate, crystals   | do    | 20   |
| Water to                        | ccs   | 1000 |

gives a transmitted density at any point along the  $\log_{10}E$  axis of the curve between the range of 0 to 2.0 which does not exceed the transmitted density obtained when an identical test layer of the emulsion (II) is developed for 4 minutes at 20° C. in the following developer (III):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate                | do    | 150  |
| Water to                        | ccs   | 1000 |

the measurements of density being made at the same points on the  $\log_{10}E$  axis of the curve, comprising simultaneously exposing the aforesaid emulsions to a lighted object or image, then treating the whole material with a developer which develops substantially only the latent image which is developable by developer (III) and then developing the whole material in a developer which develops the latent image which is developable by developer (IIa).

3. The method of selectively producing photographic images in a photographic material containing, inseparably combined and extending over the same area on a single support, two photographic emulsions having the same gamma, one of said emulsions being a light-sensitive silver halide photographic emulsion (I) a test layer of which coated on a transparent glass support upon exposure to a light intensity scale for a fixed time between  $\frac{1}{100}$  and 1 second and development for 3 minutes at 20° C. in the following developer (IIa):

|                                 |       |      |
|---------------------------------|-------|------|
| Hydroquinone                    | grams | 15   |
| N-methyl-p-aminophenol sulphate | do    | 15   |
| Sodium sulphite, anhydrous      | do    | 10   |
| Potassium bromide               | do    | 10   |
| Sodium hydroxide                | do    | 25   |
| Sodium thiosulphate, crystals   | do    | 20   |
| Water to                        | ccs   | 1000 |

gives a transmitted density at any point along the  $\log_{10}E$  axis, over a range of 3.0 starting from the threshold of the characteristic curve beginning at a density of 0.1 above fog, at least 5 times the transmitted density obtained when an identical test layer of the emulsion is developed for 4 minutes at 20° C. in the following developer (I):

|                            |       |      |
|----------------------------|-------|------|
| p-Hydroxyphenylglycine     | grams | 10   |
| Sodium carbonate, crystals | do    | 100  |
| Water to                   | ccs   | 1000 |

the measurements of density being made at the same points on the  $\log_{10}E$  axis, and the other of said emulsions being a light-sensitive silver halide photographic emulsion (II) a test layer of which coated on a transparent glass support upon exposure to a light intensity scale for a fixed time between  $\frac{1}{100}$  and 1 second and development for 4 minutes at 20° C. in the following developer (IIb):

|                                 |       |    |
|---------------------------------|-------|----|
| Hydroquinone                    | grams | 12 |
| N-methyl-p-aminophenol sulphate | do    | 3  |
| Sodium sulphite, crystals       | do    | 90 |
| Potassium bromide               | do    | 4  |

Sodium carbonate, crystals \_\_\_\_\_ grams 150  
 Sodium thiosulphate, crystals \_\_\_\_\_ do 20  
 Water to \_\_\_\_\_ ccs 1000

gives a transmitted density at any point along the  $\log_{10}E$  axis of the curve between the range of 0 to 2.0 which does not exceed the transmitted density obtained when an identical test layer of the emulsion (II) is developed for 4 minutes at 20° C. in the following developer (III):

Hydroquinone \_\_\_\_\_ grams 12  
 N-methyl-p-aminophenol sulphate \_\_\_\_\_ do 3  
 Sodium sulphite, crystals \_\_\_\_\_ do 90  
 Potassium bromide \_\_\_\_\_ do 4  
 Sodium carbonate \_\_\_\_\_ do 150  
 Water to \_\_\_\_\_ ccs 1000

the measurements of density being made at the same points on the  $\log_{10}E$  axis of the curve, comprising simultaneously exposing the aforesaid emulsions to a lighted object or image, then treating the whole material with a developer which develops substantially only the latent image which is developable by developer (III) and then developing the whole material in a developer which develops the latent image which is developable by developer (IIa).

4. The method of selectively producing photographic images in a photographic material containing, inseparably combined and extending over the same area on a single support, two photographic emulsions having the same gamma, one of said emulsions being a light-sensitive silver halide photographic emulsion (I) a test layer of which coated on a transparent glass support upon exposure to a light intensity scale for a fixed time between  $\frac{1}{100}$  and 1 second and development for 3 minutes at 20° C. in the following developer (IIa):

Hydroquinone \_\_\_\_\_ grams 15  
 N-methyl-p-aminophenol sulphate \_\_\_\_\_ do 15  
 Sodium sulphite, anhydrous \_\_\_\_\_ do 10  
 Potassium bromide \_\_\_\_\_ do 10  
 Sodium hydroxide \_\_\_\_\_ do 25  
 Sodium thiosulphate, crystals \_\_\_\_\_ do 20  
 Water to \_\_\_\_\_ ccs 1000

gives a transmitted density at any point along the  $\log_{10}E$  axis, over a range of 3.0 starting from the threshold of the characteristic curve beginning at a density of 0.1 above fog, at least 10 times the transmitted density obtained when an identical test layer of the emulsion is developed for 4 minutes at 20° C. in the following developer (I):

p-Hydroxyphenylglycine \_\_\_\_\_ grams 10  
 Sodium carbonate, crystals \_\_\_\_\_ do 100  
 Water to \_\_\_\_\_ ccs 1000

the measurements of density being made at the same points on the  $\log_{10}E$  axis, and the other of said emulsions being a light-sensitive silver halide photographic emulsion (II) a test layer of which coated on a transparent glass support upon exposure to a light intensity scale for a fixed time between  $\frac{1}{100}$  and 1 second and development for 4 minutes at 20° C. in the following developer (IIb):

Hydroquinone \_\_\_\_\_ grams 12  
 N-methyl-p-aminophenol sulphate \_\_\_\_\_ do 3  
 Sodium sulphite, crystals \_\_\_\_\_ do 90  
 Potassium bromide \_\_\_\_\_ do 4  
 Sodium carbonate, crystals \_\_\_\_\_ do 150  
 Sodium thiosulphate, crystals \_\_\_\_\_ do 20  
 Water to \_\_\_\_\_ ccs 1000

gives a transmitted density at any point along the  $\log_{10}E$  axis of the curve between the range of 0 to 2.0 which does not exceed the transmitted density obtained when an identical test layer of the emulsion (II) is developed for 4 minutes at 20° C. in the following developer (III):

Hydroquinone \_\_\_\_\_ grams 12  
 N-methyl-p-aminophenol sulphate \_\_\_\_\_ do 3  
 Sodium sulphite, crystals \_\_\_\_\_ do 90  
 Potassium bromide \_\_\_\_\_ do 4  
 Sodium carbonate \_\_\_\_\_ do 150  
 Water to \_\_\_\_\_ ccs 1000

the measurements of density being made at the same points on the  $\log_{10}E$  axis of the curve, comprising simultaneously exposing the aforesaid emulsions to a lighted object or image, then treating the whole material with a developer which develops substantially only the latent image which is developable by developer (III) and then developing the whole material in a developer which develops the latent image which is developable by developer (IIa).

5. The method of selectively producing photographic images in a photographic material containing, inseparably combined and extending over the same area on a single support, two photographic emulsions having the same gamma, one of said emulsions being a light-sensitive silver halide photographic emulsion (I) a test layer of which coated on a transparent glass support upon exposure to a light intensity scale for a fixed time between  $\frac{1}{100}$  and 1 second and development for 4 minutes at 20° C. in the following developer (IIb):

Hydroquinone \_\_\_\_\_ grams 12  
 N-methyl-p-aminophenol sulphate \_\_\_\_\_ do 3  
 Sodium sulphite, crystals \_\_\_\_\_ do 90  
 Potassium bromide \_\_\_\_\_ do 4  
 40 Sodium carbonate, crystals \_\_\_\_\_ do 150  
 Sodium thiosulphate, crystals \_\_\_\_\_ do 20  
 Water to \_\_\_\_\_ ccs 1000

gives a transmitted density at any point along the  $\log_{10}E$  axis, over a range of 3.0 starting from the threshold of the characteristic curve beginning at a density of 0.1 above fog, at least 5 times the transmitted density obtained when an identical test layer of the emulsion is developed for 4 minutes at 20° C. in the following developer (III):

Hydroquinone \_\_\_\_\_ grams 12  
 N-methyl-p-aminophenol sulphate \_\_\_\_\_ do 3  
 Sodium sulphite, crystals \_\_\_\_\_ do 90  
 Potassium bromide \_\_\_\_\_ do 4  
 55 Sodium carbonate, crystals \_\_\_\_\_ do 150  
 Water to \_\_\_\_\_ ccs 1000

the measurements of density being made at the same points on the  $\log_{10}E$  axis, and the other of said emulsions being a light-sensitive silver halide emulsion (II) a test layer of which coated on a transparent glass support upon exposure to a light intensity scale for a fixed time between  $\frac{1}{100}$  and 1 second and development for 4 minutes at 20° C. in the aforesaid developer (IIb)

gives a transmitted density at any point along the  $\log_{10}E$  axis of the curve between the range of 0 and 2.0 which does not exceed the transmitted density obtained when an identical test layer of the emulsion (II) is developed for 4 minutes at 20° C. in the aforesaid developer (III), the measurements of density being made at the same points on the  $\log_{10}E$  axis of the curve, comprising simultaneously exposing the aforesaid emulsions to a lighted object or image, then treating the whole material with a developer which develops

substantially only the latent image which is developable by developer III and then developing the whole material in a developer which develops the latent image which is developable by developer (IIa).

6. The method of selectively producing photographic images in a photographic material containing, inseparably combined and extending over the same area on a single support, two photographic emulsions having the same gamma, one of said emulsions being a light-sensitive silver halide photographic emulsion (I) a test layer of which coated on a transparent glass support upon exposure to a light intensity scale for a fixed time between  $\frac{1}{100}$  and 1 second and development for 4 minutes at 20° C. in the following developer (IIb) :

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Sodium thiosulphate, crystals   | do    | 20   |
| Water to                        | ccs   | 1000 |

gives a transmitted density at any point along the  $\log_{10}E$  axis, over a range of 3.0 starting from the threshold of the characteristic curve beginning at a density of 0.1 above fog, at least 10 times the transmitted density obtained when an identical test layer of the emulsion is developed for 4 minutes at 20° C. in the following developer (III) :

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Water to                        | ccs   | 1000 |

the measurements of density being made at the same points on the  $\log_{10}E$  axis, and the other of said emulsions being a light-sensitive silver halide emulsion (II) a test layer of which coated on a transparent glass support upon exposure to a light intensity scale for a fixed time between  $\frac{1}{100}$  and 1 second and development for 4 minutes at 20° C. in the aforesaid developer (IIb) gives a transmitted density at any point along the  $\log_{10}E$  axis of the curve between the range of 0 and 2.0 which does not exceed the transmitted density obtained when an identical test layer of the emulsion (II) is developed for 4 minutes at 20° C. in the aforesaid developer (III), the measurements of density being made at the same points on the  $\log_{10}E$  axis of the curve, comprising simultaneously exposing the aforesaid emulsions to a lighted object or image, then treating the whole material with a developer which develops substantially only the latent image which is developable by developer (III), and then developing the whole material in a developer which develops the latent image which is developable by developer (IIa).

7. A photographic material containing, inseparably combined and extending over the same area on a single support, two photographic emulsions having the same gamma, one of said emulsions being a light-sensitive silver salt photographic emulsion (I) a test layer of which coated on a transparent glass support upon exposure to a light intensity scale for a fixed time between  $\frac{1}{100}$  and 1 second and development for 3 minutes at 20° C. in the following developer (IIa) :

|                                 |       |    |
|---------------------------------|-------|----|
| Hydroquinone                    | grams | 15 |
| N-methyl-p-aminophenol sulphate | do    | 15 |
| Sodium sulphite, anhydrous      | do    | 10 |
| Potassium bromide               | do    | 10 |

|                               |       |      |
|-------------------------------|-------|------|
| Sodium hydroxide              | grams | 25   |
| Sodium thiosulphate, crystals | do    | 20   |
| Water to                      | ccs   | 1000 |

gives a transmitted density at any point along the  $\log_{10}E$  axis, over a range of 1.0 starting from the threshold of the characteristic curve beginning at a density of 0.1 above fog, at least 5 times the transmitted density obtained when an identical test layer of the emulsion is developed for 4 minutes at 20° C. in the following developer (I) :

|                            |       |      |
|----------------------------|-------|------|
| p-Hydroxyphenylglycine     | grams | 10   |
| Sodium carbonate, crystals | do    | 100  |
| Water to                   | ccs   | 1000 |

the measurements of density being made at the same points on the  $\log_{10}E$  axis, and the other of said emulsions being a light-sensitive silver salt photographic emulsion (II) a test layer of which coated on a transparent glass support upon exposure to a light intensity scale for a fixed time between  $\frac{1}{100}$  and 1 second and development for 4 minutes at 20° C. in the following developer (IIb) :

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Sodium thiosulphate, crystals   | do    | 20   |
| Water to                        | ccs   | 1000 |

gives a transmitted density at any point along the  $\log_{10}E$  axis of the curve between the range of 0 to 2.0 which does not exceed the transmitted density obtained when an identical test layer of the emulsion (II) is developed for 4 minutes at 20° C. in the following developer (III) :

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate                | do    | 150  |
| Water to                        | ccs   | 1000 |

the measurements of density being made at the same points on the  $\log_{10}E$  axis of the curve.

8. A photographic material containing, inseparably combined and extending over the same area on a single support, two photographic emulsions having the same gamma, one of said emulsions being a light-sensitive silver salt photographic emulsion (I) a test layer of which coated on a transparent glass support upon exposure to a light intensity scale for a fixed time between  $\frac{1}{100}$  and 1 second and development for 3 minutes at 20° C. in the following developer (IIa) :

|                                 |       |      |
|---------------------------------|-------|------|
| Hydroquinone                    | grams | 15   |
| N-methyl-p-aminophenol sulphate | do    | 15   |
| Sodium sulphite, anhydrous      | do    | 10   |
| Potassium bromide               | do    | 10   |
| Sodium hydroxide                | do    | 25   |
| Sodium thiosulphate, crystals   | do    | 20   |
| Water to                        | ccs   | 1000 |

gives a transmitted density at any point along the  $\log_{10}E$  axis, over a range of 3.0 starting from the threshold of the characteristic curve beginning at a density of 0.1 above fog, at least 5 times the transmitted density obtained when an identical test layer of the emulsion is developed for 4 minutes at 20° C. in the following developer (I) :

|                            |       |      |
|----------------------------|-------|------|
| p-Hydroxyphenylglycine     | grams | 10   |
| Sodium carbonate, crystals | do    | 100  |
| Water to                   | ccs   | 1000 |

the measurements of density being made at the same points on the  $\log_{10}E$  axis, and the other of

said emulsions being a light-sensitive silver salt photographic emulsion (II) a test layer of which coated on a transparent glass support upon exposure to a light intensity scale for a fixed time between  $\frac{1}{100}$  and 1 second and development for 4 minutes at 20° C. in the following developer (IIb):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Sodium thiosulphate, crystals   | do    | 20   |
| Water to                        | ccs   | 1000 |

gives a transmitted density at any point along the  $\log_{10}E$  axis of the curve between the range of 0 to 2.0 which does not exceed the transmitted density obtained when an identical test layer of the emulsion (II) is developed for 4 minutes at 20° C. in the following developer (III):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate                | do    | 150  |
| Water to                        | ccs   | 1000 |

the measurements of density being made at the same points on the  $\log_{10}E$  axis of the curve.

9. A photographic material containing, inseparably combined and extending over the same area on a single support, two photographic emulsions having the same gamma, one of said emulsions being a light-sensitive silver halide photographic emulsion (I) a test layer of which coated on a transparent glass support upon exposure to a light intensity scale for a fixed time between  $\frac{1}{100}$  and 1 second and development for 3 minutes at 20° C. in the following developer (IIa):

|                                 |       |      |
|---------------------------------|-------|------|
| Hydroquinone                    | grams | 15   |
| N-methyl-p-aminophenol sulphate | do    | 15   |
| Sodium sulphite, anhydrous      | do    | 10   |
| Potassium bromide               | do    | 10   |
| Sodium hydroxide                | do    | 25   |
| Sodium thiosulphate, crystals   | do    | 20   |
| Water to                        | ccs   | 1000 |

gives a transmitted density at any point along the  $\log_{10}E$  axis, over a range of 3.0 starting from the threshold of the characteristic curve beginning at a density of 0.1 above fog, at least 5 times the transmitted density obtained when an identical test layer of the emulsion is developed for 4 minutes at 20° C. in the following developer (I):

|                            |       |      |
|----------------------------|-------|------|
| p-Hydroxyphenylglycine     | grams | 10   |
| Sodium carbonate, crystals | do    | 100  |
| Water to                   | ccs   | 1000 |

the measurements of density being made at the same points on the  $\log_{10}E$  axis, and the other of said emulsions being a light-sensitive silver halide photographic emulsion (II) a test layer of which coated on a transparent glass support upon exposure to a light intensity scale for a fixed time between  $\frac{1}{100}$  and 1 second and development for 4 minutes at 20° C. in the following developer (IIb):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Sodium thiosulphate, crystals   | do    | 20   |
| Water to                        | ccs   | 1000 |

gives a transmitted density at any point along the  $\log_{10}E$  axis of the curve between the range of 0 to 2.0 which does not exceed the transmitted density obtained when an identical test layer of the emulsion (II) is developed for 4 minutes at 20° C. in the following developer (III):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate                | do    | 150  |
| Water to                        | ccs   | 1000 |

the measurements of density being made at the same points on the  $\log_{10}E$  axis of the curve.

15. A photographic material containing, inseparably combined and extending over the same area on a single support, two photographic emulsions having the same gamma, one of said emulsions being a light-sensitive silver halide photographic emulsion (I) a test layer of which coated on a transparent glass support upon exposure to a light intensity scale for a fixed time between  $\frac{1}{100}$  and 1 second and development for 3 minutes at 20° C. in the following developer (IIa):

|                                 |       |      |
|---------------------------------|-------|------|
| Hydroquinone                    | grams | 15   |
| N-methyl-p-aminophenol sulphate | do    | 15   |
| Sodium sulphite, anhydrous      | do    | 10   |
| Potassium bromide               | do    | 10   |
| Sodium hydroxide                | do    | 25   |
| Sodium thiosulphate, crystals   | do    | 20   |
| Water to                        | ccs   | 1000 |

gives a transmitted density at any point along the  $\log_{10}E$  axis, over a range of 3.0 starting from the threshold of the characteristic curve beginning at a density of 0.1 above fog, at least 10 times the transmitted density obtained when an identical test layer of the emulsion is developed for 4 minutes at 20° C. in the following developer (I):

|                            |       |      |
|----------------------------|-------|------|
| p-Hydroxyphenylglycine     | grams | 10   |
| Sodium carbonate, crystals | do    | 100  |
| Water to                   | ccs   | 1000 |

45. the measurements of density being made at the same points on the  $\log_{10}E$  axis, and the other of said emulsions being a light-sensitive silver halide photographic emulsion (II) a test layer of which coated on a transparent glass support upon exposure to a light intensity scale for a fixed time between  $\frac{1}{100}$  and 1 second and development for 4 minutes at 20° C. in the following developer (IIb):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Sodium thiosulphate, crystals   | do    | 20   |
| Water to                        | ccs   | 1000 |

gives a transmitted density at any point along the  $\log_{10}E$  axis of the curve between the range of 0 to 2.0 which does not exceed the transmitted density obtained when an identical test layer of the emulsion (II) is developed for 4 minutes at 20° C. in the following developer (III):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate                | do    | 150  |
| Water to                        | ccs   | 1000 |

the measurements of density being made at the same points on the  $\log_{10}E$  axis of the curve.

11. A photographic material containing, inseparably combined and extending over the same area on a single support, two photographic emulsions having the same gamma, one of said emulsions being a light-sensitive silver halide photographic emulsion (I) a test layer of which coated on a transparent glass support upon exposure to a light intensity scale for a fixed time between  $\frac{1}{100}$  and 1 second and development for 4 minutes at 20° C. in the following developer (IIb):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Sodium thiosulphate, crystals   | do    | 20   |
| Water to                        | ccs   | 1000 |

gives a transmitted density at any point along the  $\log_{10}E$  axis, over a range of 3.0 starting from the threshold of the characteristic curve beginning at a density of 0.1 above fog, at least 5 times the transmitted density obtained when an identical test layer of the emulsion is developed for 4 minutes at 20° C. in the following developer (III):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Water to                        | ccs   | 1000 |

the measurements of density being made at the same points on the  $\log_{10}E$  axis, and the other of said emulsions being a light-sensitive silver halide emulsion (II) a test layer of which coated on a transparent glass support upon exposure to a light intensity scale for a fixed time between  $\frac{1}{100}$  and 1 second and development for 4 minutes at 20° C. in the aforesaid developer (IIb) gives a transmitted density at any point along the  $\log_{10}E$  axis of the curve between the range of 0 and 2.0 which does not exceed the transmitted density obtained when an identical test layer of the emulsion (II) is developed for 4 minutes at 20° C. in the aforesaid developer (III), the measurements of density being made at the same points on the  $\log_{10}E$  axis of the curve.

12. A photographic material containing, inseparably combined and extending over the same area on a single support, two photographic emulsions having the same gamma, one of said emulsions being a light-sensitive silver halide photographic emulsion (I) a test layer of which coated on a transparent glass support upon exposure to a light intensity scale for a fixed time between  $\frac{1}{100}$  and 1 second and development for 4 minutes at 20° C. in the following developer (IIb):

|                                 |       |    |
|---------------------------------|-------|----|
| Hydroquinone                    | grams | 12 |
| N-methyl-p-aminophenol sulphate | do    | 3  |
| Sodium sulphite, crystals       | do    | 90 |

|                               |       |      |
|-------------------------------|-------|------|
| Potassium bromide             | grams | 4    |
| Sodium carbonate, crystals    | do    | 150  |
| Sodium thiosulphate, crystals | do    | 20   |
| Water to                      | ccs   | 1000 |

5 gives a transmitted density at any point along the  $\log_{10}E$  axis, over a range of 3.0 starting from the threshold of the characteristic curve beginning at a density of 0.1 above fog, at least 10 times the transmitted density obtained when an identical test layer of the emulsion is developed for 4 minutes at 20° C. in the following developer (III):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Water to                        | ccs   | 1000 |

20 the measurements of density being made at the same points on the  $\log_{10}E$  axis, and the other of said emulsions being a light-sensitive silver halide emulsion (II) a test layer of which coated on a transparent glass support upon exposure to a light intensity scale for a fixed time between  $\frac{1}{100}$  and 1 second and development for 4 minutes at 20° C. in the aforesaid developer (IIb)

25 gives a transmitted density at any point along the  $\log_{10}E$  axis of the curve between the range of 0 and 2.0 which does not exceed the transmitted density obtained when an identical test layer of the emulsion (II) is developed for 4 minutes at 20° C. in the aforesaid developer (III), the measurements of density being made at the same points on the  $\log_{10}E$  axis of the curve.

30

35

EDWARD BOWES KNOTT.  
GUY WILLIAM WILLIS STEVENS.

#### REFERENCES CITED

The following references are of record in the file of this patent:

#### UNITED STATES PATENTS

|    |           |          |               |
|----|-----------|----------|---------------|
| 45 | Number    | Name     | Date          |
|    | 1,857,083 | Harris   | May 3, 1932   |
|    | 1,930,141 | Capstaff | Oct. 10, 1933 |
|    | 1,956,230 | Schmidt  | Apr. 24, 1934 |
| 50 | 2,029,946 | Schmid   | Feb. 4, 1936  |
|    | 2,197,994 | Butement | Apr. 23, 1940 |

#### OTHER REFERENCES

Mees, "The Theory of the Photographic Process," published 1942 by The MacMillan Co., New York; pages 150-152, 166-171, 196, 294-297 and 301.

55 Bullock, "Chemical Reactions of The Photographic Latent Image," vol. I, published by Eastman Kodak Co., Rochester, New York, 1927; pages 15, 20, 22, 28, 30, 31, 47, 48, 50, 52, 72, 73, 80-85.

60 Wall, "Photographic Emulsions," published by Amer. Phot. Pub. Co., Boston, 1929, pages 52, 53 and 135 to 137.

65